



US005238505A

**United States Patent** [19]**Kaiser**[11] **Patent Number:** **5,238,505**[45] **Date of Patent:** \* Aug. 24, 1993

[54] **METHOD FOR APPLYING  
TELLURIUM-CONTAINING COATINGS TO  
METALLIC SURFACES USING ORGANIC  
ACIDS**

[75] Inventor: **Herbert J. Kaiser**, St. Louis, Mo.

[73] Assignee: **Calgon Corporation**, Pittsburgh, Pa.

[\*] Notice: The portion of the term of this patent  
subsequent to Feb. 18, 2009 has been  
disclaimed.

[21] Appl. No.: **772,396**

[22] Filed: **Oct. 7, 1991**

[51] Int. Cl.<sup>5</sup> ..... **C23C 22/07**

[52] U.S. Cl. ..... **148/259; 148/261**

[58] Field of Search ..... **148/259, 270, 261**

[56] **References Cited**

**U.S. PATENT DOCUMENTS**

4,149,909 4/1979 Hamilton .

4,224,301 9/1980 Washall .

4,256,912 2/1991 Wolsky et al. .

4,391,855 7/1983 Geeck .  
4,595,424 6/1986 Hacias .  
4,639,295 1/1987 Miyamoto et al. .  
4,713,121 12/1987 Zurilla et al. .  
4,929,739 5/1990 Sredni et al. .  
5,089,349 2/1992 Kaiser .

**OTHER PUBLICATIONS**

The Merck Index (Tenth Edition) pp. 8970-8971.  
"Studies on Complex Formation of Tellurium with  
Tartaric, Citric and Malic Acids", S. Prasad and K.  
Pathak, Jour. & Proc. Inst. Chem. vol. XXXVIII (Nov.  
1966) pp. 260-261.

*Primary Examiner*—Sam Silverberg

*Attorney, Agent, or Firm*—W. C. Mitchell; C. M. Caruso

[57] **ABSTRACT**

Improved tellurium-containing coating compositions  
and a method for applying a tellurium-containing coating  
to a metallic surface characterized by the presence  
of tellurium and an organic acid solubilizing agent.

**4 Claims, No Drawings**

**METHOD FOR APPLYING  
TELLURIUM-CONTAINING COATINGS TO  
METALLIC SURFACES USING ORGANIC ACIDS**

**BACKGROUND OF THE INVENTION**

This invention relates to improved tellurium compositions and a method for applying tellurium coatings to metallic surfaces. These coating compositions are characterized by the presence of tellurium and an organic acid solubilizing agent.

As used herein, the term "coating" refers to a material bonded to the surface of a metal which differs chemically from the metal itself. A particular example of a coating is a phosphate-based conversion coating. Such a coating is formed by chemical interaction between a phosphate-containing coating composition and the metal substrate being treated.

Conversion coatings are used to enhance the corrosion resistance of treated metal surfaces and to improve the adherence of paints and other coatings to these surfaces. As practiced in the art, conversion coatings are generally applied to metallic surfaces as iron phosphate, zinc phosphate or manganese phosphate. For example, a conversion coating may be produced by contacting a metal surface with a composition comprising a phosphate source, an acid and an accelerator. Typical accelerators used for this purpose include molybdenum, vanadium, nickel and tungsten salts.

Prior to application of a conversion coating, the metallic surface to be treated is generally cleaned to remove oil, grease, and other impurities. These impurities may act as mechanical barriers to conversion coating compositions or solutions, and can either interfere with or completely prevent adherence of the conversion coating to the metallic surface being treated.

After cleaning, the metallic surface is typically contacted with a conversion coating solution which comprises an acid, a phosphate source, an oxidizer and an accelerator. The surface is then generally rinsed with water to remove unreacted reagents and phosphate salts. Finally, a chromate, nitrate, or acid sealing rinse may be applied to the surface being treated, prior to painting.

Several disadvantages inherently plague conventional conversion coating methods, such as iron phosphate coating methods. Key among these is that iron phosphate processes generally produce coatings which provide less corrosion resistance than zinc phosphate coating processes. Since zinc phosphate processes are generally more complex and more costly to utilize, and are environmentally undesirable, there is a long-felt need in the art for a convenient, inexpensive method of providing corrosion-resistant conversion coatings. This need is met by the instant method and compositions.

It is therefore an object of this invention to provide improved tellurium compositions and an improved method for applying a uniform, durable tellurium coating to a metallic surface which provides corrosion resistance to the substrate being treated. This object is accomplished by utilizing tellurium coating compositions which contain a tellurium ion source and a solubilizing agent selected from the group consisting of  $\alpha$ -substituted organic acids to form a coating characterized by the presence of tellurium. Particular examples of the instant solubilizing agents include, but are not limited to, hydroxyacetic acid, tannic acid, tartaric acid, citric acid, 2,6-pyridine-dicarboxylic acid, lactic acid,

glucono  $\delta$ -lactone (gluconic acid), 2-puroic acid, thiophene-2-carboxylic acid, 2,3-pyridine dicarboxylic acid, phosphonoacetic acid, thiophene-2-acetic acid and mercaptoacetic acid.

5 Any metallic surface can be treated according to the instant invention, including but not limited to galvanized surfaces, stainless steel surfaces, mild steel surfaces and aluminum surfaces.

10 This and other objects of the instant invention are accomplished by use of the instant compositions and the method disclosed herein. The instant coating compositions and method allow the application of uniform tellurium coatings to metallic surfaces, particularly in the mid-pH range. The method can be utilized at any temperature up to boiling, and the resulting coating provides corrosion resistance to the substrate. The instant coatings also generally improve the appearance of paints and other coatings subsequently applied to treated metallic surfaces.

15 The MERCK INDEX, Tenth Edition, discloses that tellurium is a reagent which produces a black finish on silverware.

20 U.S. Pat. No. 4,713,121 discloses phosphate conversion coatings which contain first and second divalent metal elements, such as cobalt and zinc.

25 U.S. Pat. No. 4,391,855 discloses a coating method which utilizes compositions containing a powdered metal dispersed in a bonding material as a corrosion inhibitor.

30 U.S. Pat. No. 4,149,909 discloses the use of chlorates and bromates as accelerators and hydroxylamine sulfate as a reducing agent in phosphatizing compositions used to produce iron phosphate coatings.

35 U.S. Pat. No. 4,595,424 discloses phosphate coating solutions for use on zinc surfaces which contain a phosphate ion source, a zinc and/or manganese ion source and a complex of fluoride ions.

40 U.S. Pat. No. 4,634,295 discloses a method for improving corrosion resistance of metal substrates which requires application of a direct current to a previously zinc-phosphated metal surface in an acidic solution containing zinc, phosphate and chloride ions.

45 Copending application U.S. application Ser. No. 361,087 discloses tellurium compositions and methods for applying the same to metallic surfaces. Copending application U.S. Ser. No. 739,010 discloses the use of  $\alpha$ -substituted organic acids to solubilize tellurium.

**SUMMARY OF THE INVENTION**

This invention relates to improved tellurium coating compositions and to an improved method for applying a tellurium coating to a metallic surface, wherein the method and compositions are characterized by the use and/or presence of a tellurium ion source and a tellurium solubilizing agent selected from the group consisting of  $\alpha$ -substituted organic acids.

**DETAILED DESCRIPTION OF THE  
INVENTION**

The instant invention is directed to a method for applying a coating to a metallic surface which comprises:

(A) contacting said metallic surface with an effective amount of an aqueous coating composition which comprises:

(a) water

- (b) about 0.1 to about 100,000 ppm, based on the weight of (a) of tellurium ions;
- (c) about 0.1 to about 100,000 ppm, based on the weight of (a) of an  $\alpha$ -substituted organic acid;
- (d) optionally, about 0.1 to about 400,000 ppm, based on the weight of (a) of phosphate ions; and
- (e) optionally, about 0.1 to about 200,000 ppm, based on the weight of (a) of an oxidizer; and

(B) Optionally, rinsing and drying said metallic surface. 10

Relative to this method, the term "effective amount" refers to that quantity of coating composition necessary to provide intimate contact between the metal surface to be coated and the coating composition for a time adequate to allow a coating characterized by the presence of tellurium to bond to the metallic surface being treated. 15

In the instant water-based compositions, an  $\alpha$ -substituted organic acid is used as a tellurium solubilizing agent. As disclosed in copending U.S. application Ser. No. 739,010,  $\alpha$ -substituted carboxylic acids solubilize tellurium over the entire pH range. This enables substrates to be coated using tellurium coating compositions in the mid pH range. Thus, the instant coating compositions may be formulated at a pH where tellurium is soluble. The pH of the coating compositions can then be adjusted to the mid-pH range so that the coating may be applied more conveniently and safely. As used herein, the term "mid pH range" is from about 2.5 to about 11.0, preferably from about 3.0 to about 9.0. 20

The tellurium ion source provides the tellurium present in the coating formed on the substrate. Optionally, phosphate ion sources and/or oxidizers may be used. Phosphates and oxidizers facilitate preparation of the metallic substrate. One or more acids may also be present. Acids are believed to facilitate the bonding of the tellurium coating to the substrate. Hydrochloric acid and sulfuric acid are preferred. 25

In general terms, it is believed that the instant solubilizing agents comprise a class of organic acids which contain an element or a functional group of sufficient electron density to chelate, complex or react with tellurium on the carbon alpha to the acid group. Such agents have the following general structure:



wherein:

X is an element or functional group of sufficient electron density to chelate or react with tellurium. Particular examples of X include, but are not limited to, functional groups with heteroatoms such as O, S, N. Preferred examples include OH and SH. 55

R<sub>1</sub> and R<sub>2</sub>, which may be the same or different, include hydrogen, straight or branched alkyl groups, aryl groups, substituted alkyl groups and substituted aryl groups.

Also, alpha-substituted heterocyclic organic acids 65 function to maintain tellurium solubility. Examples of such compounds include, but are not limited to, the pyridine dicarboxylate analogues shown below:



2,6-Pyridine Dicarboxylic Acid



2,3-Pyridine Dicarboxylic Acid

Both the 2,6-dicarboxylic acid and the 2,3-dicarboxylic acid maintain the solubility of the tellurium.

Other examples of heterocyclic compounds which maintain tellurium solubility include 2-furoic acid and thiophene-2-carboxylic acid, whose structures are shown below.



2-Furoic Acid



Thiophene-2-Carboxylic Acid

The preferred  $\alpha$ -substituted organic acid solubilizing agents for use in the instant method are selected from the group consisting of hydroxyacetic acid, tannic acid, tartaric acid, citric acid, 2,6-pyridine dicarboxylic acid, lactic acid, glucono  $\alpha$ -lactone (gluconic acid), 2-pyroic acid, thiophene-2-carboxylic acid, thiophene-2-acetic acid, mercaptoacetic acid and mixtures thereof. These preferred compounds are believed to be commercially available from Sigma Chemical Company.

More preferred solubilizing agents are compounds selected from the group consisting of hydroxyacetic acid, tartaric acid and citric acid. Citric acid is believed to be the most preferred solubilizing agent.

Additionally, effective amounts of surfactants may be added for cleaning, penetration and/or wetting purposes, and an effective amount of a fluoride source may be added for use on galvanized or aluminum surfaces. Other conventional additives used in conversion compositions, such as chelants, may also be added.

The instant invention is also directed to compositions comprising:

- (a) water;
- (b) about 0.1 to about 400,000 ppm, based on the weight of (a), of phosphate ions;
- (c) about 0.1 to about 100,000 ppm, based on the weight of (a), of a tellurium; ion source; and
- (d) about 0.1 to about 100,000 ppm, based on the weight of (a), of an  $\alpha$ -substituted organic acid.

The instant compositions provide coatings which are characterized by the presence of tellurium. These coatings generally enhance the resistance to corrosion of treated metallic surfaces and improve the adherence of paints and other coatings to these surfaces. Prior to the application of the instant coatings, the surface to be coated is generally cleaned using some combination of chemical additives, mechanical scrubbing and water rinsing. Conventional conversion coating compositions, such as iron phosphate coating compositions, generally contain metals such as molybdenum, vanadium, nickel and/or tungsten salts to accelerate the coating process and to provide even, adherent coatings.

An essential component of the instant compositions is an  $\alpha$ -substituted organic acid solubilizing agent. The preferred  $\alpha$ -substituted organic acid solubilizing agents for use in the instant compositions are selected from the

group consisting of hydroxyacetic acid, tannic acid, tartaric acid, citric acid 2 6-pyridine dicarboxylic acid lactic acid, glucono  $\delta$ -lactone (gluconic acid), 2-puroic acid, thiophene-2-carboxylic acid, thiophene-2-acetic acid mercaptoacetic acid and mixtures thereof.

More preferred solubilizing agents are compounds selected from the group consisting of hydroxyacetic acid, tartaric acid and citric acid. Citric acid is believed to be the most preferred solubilizing agent.

The organic acid solubilizing agents solubilize tellurium ions over a wide pH range, making it possible to apply tellurium coatings at moderate pH's. In the absence of an  $\alpha$ -substituted organic acid or other solubilizing agent, tellurium is generally insoluble at pH's below about 2.5 and greater than about 11.0.

Optionally, any source of phosphate ions can be used in the instant compositions and method, including but not limited to phosphoric acid and phosphate salts, such as ammonium, potassium, lithium, or sodium salts of ortho phosphoric acid or pyro phosphoric acid. For example, suitable phosphate salts include but are not limited to mono potassium ortho phosphate, dipotassium ortho phosphate, tripotassium ortho phosphate, mono sodium ortho phosphate, disodium ortho phosphate, trisodium ortho phosphate, hemisodium ortho phosphate, mono ammonium ortho phosphate, diammonium ortho phosphate, triammonium ortho phosphate, lithium ortho phosphate, sodium tripolyphosphate, tetrasodium pyrophosphate, disodium pyrophosphate, sodium hexametaphosphate, sodium ammonium pyrophosphate, sodium octametaphosphate, and sodium heptametaphosphate. The preferred sources of phosphate ions are trimetaphosphates, orthophosphates, hexametaphosphates and tripolyphosphates. The most preferred phosphate ion source is sodium trimetaphosphate. The instant coating compositions may contain from about 0.1 up to about 400,000 ppm, based on the total water in the coating composition, of phosphate ions, on an active basis. Preferably, these compositions contain about 1 to about 200,000 ppm of phosphate ions. It is believed that phosphate ions assist in maintaining tellurium and/or selenium solubility. The phosphates may also act as chelants and sludge reducers.

The instant coating compositions may optionally contain about 0.1 to about 200,000 ppm of an oxidizer, based on weight of water in the coating composition. Preferably, they contain about 1.0 to about 100,000 ppm of an oxidizer. Any oxidizer can be used. The preferred oxidizers are selected from the group consisting of chloride and nitrate salts. The most preferred oxidizers are sodium chloride and sodium nitrate.

The instant coating compositions contain at least about 0.1 ppm of tellurium ions (on an active basis) with the upper limit set by tellurium solubility, based on the weight of water in the coating composition. Preferably about 0.1 to about 100,000 ppm, and most preferably about 1 to about 50,000 ppm of tellurium ions are present. Any source of tellurium ions may be used. Preferred tellurium ion sources are the oxides of tellurium and salts of telluric acid or tellurous acid. The most preferred sources of tellurium ions are tellurium oxide and salts of telluric acid.

The balance of the instant composition is water, though additional agents may be used. For example, acids, surfactants, fluoride ion sources and chelants may also be desirable.

An effective amount of a heavy metal catalyst can also optionally be used in the compositions of the instant

invention. Such catalysts include, but are not limited to, compounds of such metals as vanadium, titanium, zirconium, tungsten, and molybdenum. The preferred catalysts are sodium molybdate and ammonium metavanadate. In combination with or in place of these heavy metal catalysts, additional accelerators such as acid-soluble salts of nickel, cobalt, magnesium, sodium and calcium may be utilized in the compositions of the instant invention. Typical anions for these salts include but are not limited to nitrates, nitrites and chlorates.

An effective amount of a chelating agent can also optionally be used in the instant invention. Such agents include, but are not limited to thiourea, ethylene diamine tetraacetic acid, and nitrilotriacetic acid. The preferred chelant is ethylene diamine tetraacetic acid (hereinafter EDTA). The EDTA component of the composition may be of any suitable grade. For example, commercially available solutions which are 39%, by weight, may be used. It is noteworthy that some acids, such as citric acid and EDTA, are well-known chelants.

The compositions of the present invention must contact the metal being treated for an effective amount of time. As used herein, "effective amount of time" means that amount of time required for the composition to contact and to react with the metallic surface being treated so as to produce a uniform, adherent coating. Preferably, the contact time should be about 1-60 minutes, more preferably about 1-30 minutes and most preferably, about 1-5 minutes. Contact between the coating composition and the metal surface can be made to occur by any known method, including but not limited to spraying and immersion techniques. While application temperature is not believed to be critical, a practical upper limit is the boiling temperature of the aqueous coating composition. However, the preferred contact temperature is less than about 120° F.

|                      | Weight Percent<br>(Active Basis) |
|----------------------|----------------------------------|
| Citric Acid          | 2-20                             |
| Phosphate Ion Source | 1-20                             |
| Oxidizer             | 0.5-10                           |
| Tellurium            | 0.01-3                           |
| Water                | Balance                          |

Optionally, the compositions of the present invention may contain about 0.1% to 5%, by weight, of a heavy metal catalyst and about 0.1% to 10%, by weight, of a chelating agent. Also, at least 0.1, by weight, preferably about 0.1% to about 10%, by weight, of a fluoroborate compound may be used to provide fluoride ions to etch the metallic surface being treated.

The compositions of the instant invention may be prepared by conventional mixing or blending techniques in a mix tank. Agitation is desirable. Order of addition is not believed to be critical. However, the solubilizing agent and the tellurium ion source should generally be added prior to any pH adjustment step.

The compositions of the instant invention may be applied to a metallic surface by any known method of application including but not limited to spray and immersion techniques. Optionally, the coating composition can then be rinsed and allowed to dry, which leaves the coating behind.

The process described herein may be followed by or may additionally comprise other steps conventionally used in preparing metallic surfaces for painting, includ-

ing but not limited sealing the coated metallic surface with chromic or non-chromic based materials.

#### EXAMPLE

The following example further demonstrates the instant invention. This example is not intended to limit the invention in any way.

##### Tellurium-Based Phosphatizer Using Tartaric Acid

| Ingredient              | Weight Percent of Composition |
|-------------------------|-------------------------------|
| Water                   | 64.52                         |
| Sodium Hydroxide (50%)  | 8.00                          |
| Tellurium Dioxide       | 0.48                          |
| Tartaric Acid           | 6.00                          |
| Glacial Acetic Acid     | 4.00                          |
| Sodium Trimetaphosphate | 5.40                          |
| Sodium Chloride         | 1.40                          |
| d-Glucose Monohydrate   | 2.70                          |
| Sodium Sulfate          | 7.50                          |

The above ingredients were added in the order they are listed. The final formulation was a clear, stable solution having a pH of 4.85.

What is claimed is:

1. A composition for applying a coating to a metallic surface comprising:

- (a) water;
- about 0.1 to about 400,000 ppm, based on the weight of (a), of phosphate ions;
- (c) about 0.1 to about 100,000 ppm, based on the weight of (a), of a tellurium ion source;
- (d) about 0.1 to about 100,000 ppm, based on the weight of (a), of an  $\alpha$ -substituted organic acid.

2. The composition of claim 1, wherein the pH of said composition is adjusted to the mid-pH range.

3. The composition of claim 1, wherein said  $\alpha$ -substituted organic acid is selected from the group consisting of organic acids which contain an element or functional group of sufficient electron density to chelate, complex or react with tellurium on the carbon to the acid group.

4. The composition of claim 2, wherein said  $\alpha$ -substituted organic acid is selected from the group consisting of organic acids which contain an element or functional group of sufficient electron density to chelate, complex or react with tellurium on the carbon to the acid group.

\* \* \* \* \*